

Patented Mar. 18, 1941

2,234,955

# UNITED STATES PATENT OFFICE

2,234,955

## NICKEL ALLOYS AND PROCESS OF TREATING THE SAME

Clarence George Bieber and Mortimer Pierce  
Buck, Huntington, W. Va., assignors to The  
International Nickel Company, Inc., New York,  
N. Y., a corporation of Delaware

No Drawing. Application January 28, 1939.  
Serial No. 253,350

7 Claims. (Cl. 148—13)

The present invention relates to improved age hardenable nickel alloys and age-hardened articles of manufacture made thereof, and to a process for heat treating such alloys, and more particularly to improved corrosion-resistant age hardenable nickel-copper-aluminum alloys and improved articles made thereof.

It is well known that corrosion-resistant alloys of nickel and copper possessed improved properties when aluminum was present in amounts up to 17%. Thus, in United States Patent No. 1,572,744 to P. D. Merica, a nickel-copper alloy was described which contained from 1% to 17% aluminum and possessed increased hardness and tensile strength while retaining the ability to resist corrosion. It was later found that the physical properties of the alloys could be greatly improved if the alloys were subjected to a heat treatment. Thus, United States Patents Nos. 1,755,554 to 1,755,557 to Mudge relate to the method of heat treating nickel-copper-aluminum alloys. The resulting improvement in the properties is attributed to an age-hardening effect.

We have now discovered that articles of manufacture made of these corrosion resisting nickel-copper-aluminum alloys possesses further improved properties when controlled and critical amounts of titanium are incorporated in the alloy.

It is an object of the present invention to provide age hardened articles of manufacture made of improved nickel-copper-aluminum alloys, of the type described in the aforementioned Merica and Mudge patents, containing critical and controlled amounts of titanium and possessing superior hot ductility in the commercial hot working range of about 1400° F. to about 2300° F. without adverse effect on the mechanical properties of the alloys or the age hardening treatment necessary to produce the same.

It is another object of the present invention to provide improved age-hardened articles of manufacture made of corrosion-resistant carbon-bearing nickel-copper-aluminum-titanium alloys, said aluminum and titanium being present in controlled amounts and said articles possessing improved properties.

It is a further object of the present invention to provide improved, age-hardened articles of manufacture made of corrosion-resistant carbon-bearing nickel-copper-aluminum alloys which contain controlled and critical amounts of titanium, said articles of manufacture being less susceptible to loss of strength and/or ductility after exposure for long periods of time at elevated temperatures.

The invention contemplates improved corrosion and wear-resistant articles of manufacture made of certain carbon-bearing nickel-copper-aluminum-titanium alloys and characterized by

the ability to retain high properties at elevated temperatures, e. g., at steam temperatures of about 1000° F.

The invention further contemplates improved age hardened carbon-bearing nickel-copper-aluminum-titanium alloys characterized by improved hot ductility in the commercial hot working range of temperatures and improved physical properties in the age hardened condition.

It is within the contemplation of the present invention to provide improved age hardenable nickel-copper-aluminum alloys containing critical and controlled amounts of titanium and characterized by improved hot ductility in the hot working range and improved physical properties in the age hardened condition.

Furthermore, it is also within the contemplation of the present invention to provide an improved process for age hardening the alloys of the present invention and other age hardenable nickel products, including nickel-copper-aluminum alloys, to impart further improved properties to the alloys, said process involving special and controlled aging operations.

It is also within the contemplation of the present invention to provide an improved process for age hardening the alloys of the present invention and other age hardenable nickel products in which the necessity of a quenching operation prior to aging is eliminated.

Other objects and advantages of the invention will become apparent to those skilled in the art from the following description.

In general, the invention provides improved age-hardened articles of manufacture made of nickel-copper-aluminum-titanium alloys such as those alloys wherein the ratio of nickel to copper is in the neighborhood of two parts nickel to one part copper.

Suitable alloys in accordance with the present invention are those having compositions within the ranges given in Table I.

Table I

| Element  | Percentage |
|----------|------------|
| Nickel   | 50-85      |
| Copper   | 10-45      |
| Aluminum | 2-4        |
| Titanium | 0.25-1.0   |
| Carbon   | 0.05-0.3   |

In addition, silicon, manganese and iron may be present in the alloy within the ranges of about 0.05% to about 1% silicon, about 0.05% to about 2% manganese and about 0.05% to about 10% iron.

We have discovered that articles manufactured from these alloys are particularly improved when titanium is present in the alloys in

amounts of about 0.4% to about 0.75% and when the aluminum is restricted to amounts ranging from about 2.3% to about 3.4%. The articles can be heat-treated in accordance with the technique developed by Mudge and described in the United States Patents 1,755,554 to 1,755,557, inclusive. Generally speaking, the articles are heat-treated subsequent to mechanical working and forming operations. Under certain conditions the articles may be heat treated before the final operations. For example, fine spring wires may be cold drawn after the hardening heat treatment, since this procedure develops the highest physical properties attainable in the material. It also produces finished material with a higher luster than can be developed in material which is heat treated after cold drawing. Finish machining may also be carried out after heat treatment to eliminate any discoloration and warping which occur during heat treatment. Heat treated material may be subjected to subsequent machining, stamping, or other fabricating operations whenever necessary.

Hot rolled material having the composition contemplated by the present invention will heat treat to Brinell hardnesses in excess of about 265, and about 300 Brinell represents an average value. Cold drawn or cold worked material in smaller sections, for example up to about one inch in sectional thickness, generally heat treats to Brinell hardness values of about 325 or more. Larger cold worked sections generally do not heat treat to much higher hardness values than hot rolled material of the same sections.

In carrying the present invention into practice, the new articles of manufacture are preferably made of corrosion-resistant nickel-copper alloys having compositions within the more specific ranges given in Table II. Prior to the present invention, the preferred alloys of nickel and copper contained about 3.75% of aluminum and small amounts of carbon, manganese, iron, etc. While satisfactory properties can be obtained when the composition is within the ranges given in Table I, it is generally preferred to maintain the composition as near the more specific ranges given in Table II as variations due to commercial production methods will allow. In this manner the best results are assured. Variations from the preferred ranges due to commercial production methods are generally within the ranges given in Table I.

Table II

| Element       | Percentage   |
|---------------|--------------|
| Nickel.....   | 63.0 to 70.0 |
| Copper.....   | 25.0 to 35.0 |
| Aluminum..... | 2.7 to 3.1   |
| Titanium..... | 0.4 to 0.6   |
| Carbon.....   | 0.18 to 0.20 |

In commercial practice, silicon, manganese and iron are often present and usually fall within the range of about 0.2% to about 0.4% silicon, about 0.25% to about 0.5% manganese and about 0.2% to about 1% iron.

The aluminum and titanium present in the alloys are considered as major elements in the age-hardening process while the carbon and to some extent the silicon are considered as minor elements in this process. Iron and manganese apparently affect the base alloy only. When nickel is said to constitute the "balance" or when we say that the "balance is substantially all"

nickel, we include within the expression minor constituents and impurities such as cobalt, silicon, manganese, iron, sulfur, phosphorus and other elements commonly present in commercial products. Magnesium is generally not present, as it has been found that magnesium is detrimental to the hot ductility of the materials contemplated by the present invention. We have found that the titanium content is critical and must be at least 0.25% and less than 1% of the alloy. To be of commercial value, the alloys should be capable of heat treatment to a minimum hardness of about 265 to 300 Brinell without cold working and should possess satisfactory hot ductility. Titanium in amounts less than 0.25% produces results which are not appreciably better than that obtained in material containing aluminum only. An alloy containing approximately 2.75% aluminum and 0.50% titanium will readily produce high hardnesses of commercial value. With decreased aluminum contents, the titanium is increased to 0.75% or more. Materials having titanium contents of 1% or more develop a pronounced tendency towards "center splitting" during rolling into small rods, etc. This "center splitting" may be considered as a manifestation of poor hot ductility. Consequently, an excess of titanium destroys the beneficial results obtained by a small amount of the element. In addition, no benefits are derived from increasing the titanium contents above 0.75% to 1% while titanium contents of 1% or more are also very inefficient functionally. Titanium contents above 1.0% require twice as much titanium to produce the same effect as at a level of about 0.5% titanium. The ineffectiveness, or lesser effectiveness, of titanium, when added in amounts in excess of about 0.5% is illustrated in Table III. This table sets forth the hardness of similar materials comprising principally nickel and copper in the ratio of about two to one and containing 2.75% aluminum and various amounts of titanium, as heat treated to maximum hardness without any cold working effect.

Table III

|                        |      |      |      |        |
|------------------------|------|------|------|--------|
| Per cent aluminum..... | 2.75 | 2.74 | 2.75 | 2.72   |
| Per cent titanium..... | None | 0.51 | 0.73 | 1.01   |
| Brinell hardness.....  | 174  | 285  | 302  | 311 50 |

It will be observed from Table III that very little increase in hardness is obtained by increasing the titanium beyond about 0.5% to about 0.75%. The gain in hardness due to the presence of 0.5% titanium is much greater proportionally than the gain due to additional amounts of titanium and, further, the gain in hardness decreases sharply as the total titanium content increases. The high cost of titanium is another serious objection to the use of this element in quantities greater than absolutely necessary. The most economic utilization of titanium is secured when present in quantities of about 0.4% to about 0.6%. A considerable portion of the physical properties of the materials contemplated by the present invention are due to the presence of carbon. It is therefore preferred to maintain the carbon content at the highest level that is possible without sacrificing hot malleability, since the higher carbon contents impart increased strength and hardness. Whereas carbon is highly detrimental in high titanium alloys of nickel and copper, it is highly beneficial and even necessary in material made in accordance with the present invention.

Table IV compares the behavior of carbon in heat treated material comprising principally nickel and copper in the ratio of approximately two parts nickel to one part copper and containing high titanium with similar material containing low titanium and high aluminum.

Table IV

| 10 | Percent C | Percent Ti | Percent Al | Brinell hardness |
|----|-----------|------------|------------|------------------|
| 15 | None      | 3.63       | -----      | 302              |
| 20 | 0.20      | 3.63       | -----      | 156              |
| 25 | None      | 0.53       | 2.93       | 241              |
| 30 | 0.20      | 0.53       | 2.93       | 302              |

The behavior of the high titanium material in the presence of carbon is believed to be explained by the formation of an inert titanium carbide which decreases the hardening efficiency of the titanium. The fact that the presence of carbon increases the physical properties of material made in accordance with the present invention indicates that inert titanium carbides do not form as in the case of the high titanium material and that carbon is highly beneficial in low titanium material.

The advantageous use of restricted amounts of titanium and aluminum in the alloys does not conflict with the heat treatment technique described in the Mudge patents. Titanium and aluminum in amounts within the contemplation of the present invention offer marked improvements in the age hardening properties of the alloys. The hardness and strength of articles made of the old nickel-copper-aluminum alloys are increased about 10 to 15% or more without appreciable decrease in ductility when made in accordance with the present invention. The alloys used in the present invention may be heat treated in the same manner as the nickel-copper-aluminum alloys but are preferably treated in accordance with an improvement thereover which will be described more fully hereinafter.

Articles manufactured in accordance with the present invention are also less susceptible to loss of strength and/or ductility after exposure for long periods of time at temperatures of approximately 500° F. to approximately 1100° F. Such articles retain their high properties at elevated temperatures, for instance, at steam temperatures of about 1000° F. Table V compares the properties of prior titanium-free material with our improved titanium bearing material in the as heat treated condition and after heat treating and aging for 18 months at 800° F.

Table V

| 60 | Material         | Condition    | Y. P. | B. S. | Percent El. | Percent R. A. |
|----|------------------|--------------|-------|-------|-------------|---------------|
| 65 | Titanium-free    | Heat treated | 86.5  | 148.3 | 25.0        | 46.3          |
|    | Do.              | Heat aged    | 95.0  | 153.0 | 17.5        | 24.4          |
| 70 | Titanium-bearing | Heat treated | 97.8  | 150.5 | 28.0        | 45.4          |
|    | Do.              | Heat aged    | 113.5 | 165.0 | 24.0        | 38.8          |

Y. P. = yield point in thousand pounds per square inch.  
B. S. = breaking strength in thousand pounds per square inch.  
Percent El. = percent elongation in 2 inches.  
Percent R. A. = percent reduction of area.

The improved high temperature stability of the titanium-bearing material is particularly noticeable in the loss of ductility in the older titanium free material. The titanium-bearing material also possesses a higher yield point and breaking

strength than the prior material. Under certain conditions the titanium-free material exhibits marked decreases in strength after being subjected to elevated temperatures for long periods of time.

The titanium-bearing material possesses improved hot ductility without detrimental effect upon the mechanical properties or the method of heat treatment necessary to procure the mechanical properties. The alloys of the present invention possess improved hot ductility within the hot working range of about 1400° F. to about 2300° F. The differences in hot ductilities between the titanium-free and the titanium-bearing alloys contemplated by the present invention are very pronounced. For example, a titanium-bearing alloy had a hot malleable range of about 800° F. or more, whereas a titanium-free alloy had a hot malleable range of only about 400° F. Data from typical melts are given in Table VI.

Table VI

| 25               | Material     | Hot malleable range |
|------------------|--------------|---------------------|
| Titanium-free    | -----        | ° F.                |
| Titanium-bearing | 1900 to 2300 | 1500 to 2300        |

The difference in hot malleability between the titanium-free material and the titanium-bearing material represents the difference between material which is not commercially malleable and material which is commercially malleable. Articles of manufacture made in accordance with our invention are also corrosion-resistant, oxidation-resistant, wear-resistant, hard, strong, machinable, non-magnetic, etc.

In accordance with the present invention, improved articles of manufacture, for example, valve parts, pump pistons, turbine blades, etc., are satisfactorily made of the alloy given in Table VII.

Table VII

| 50        | Element    | Percentage |
|-----------|------------|------------|
| Nickel    | About 66.0 | 50         |
| Copper    | About 29.0 |            |
| Aluminum  | About 3.0  |            |
| Titanium  | About 0.5  |            |
| Carbon    | About 0.2  |            |
| Silicon   | About 0.25 |            |
| Manganese | About 0.40 |            |
| Iron      | About 0.65 | 55         |

The material is mechanically worked as desired into the required shape and heat treated to age-harden the material. Preferably the heat treatment is conducted in accordance with the improved methods discussed more fully hereinafter, the best heat treatment being dependent upon the finishing temperature of the mechanical treatment and the amount of cold work imparted to the material.

Some of the advantages of the present invention are illustrated in Tables VIII and IX which give the composition and properties of a titanium-free heat-treated alloy containing 3.00% aluminum and of another made in accordance with a preferred embodiment of the present invention and containing 3.01% aluminum and 0.53% titanium. The improved properties of the titanium-bearing material are readily observed.

Table VIII

| 5  | No. | Composition in percent |            |            |            |           |            |            |            |            |
|----|-----|------------------------|------------|------------|------------|-----------|------------|------------|------------|------------|
|    |     | Percent Ni             | Percent Cu | Percent Al | Percent Ti | Percent C | Percent Si | Percent Mn | Percent Fe | Percent Mg |
| 10 | A   | 66.15                  | 29.90      | 3.00       | None       | 0.15      | 0.25       | 0.25       | 0.30       | None       |
|    | B   | 65.75                  | 29.72      | 3.01       | 0.53       | 0.16      | 0.25       | 0.23       | 0.32       | None       |

Table IX

| 15 | No. | Hardening heat treatment                                 | Physical properties |         |       |               |             |
|----|-----|----------------------------------------------------------|---------------------|---------|-------|---------------|-------------|
|    |     |                                                          | Y. P.               | T. S.   | B. H. | R. A. percent | El. percent |
| 20 | A   | 1100° F. for 16 hrs. followed by slow cooling to 900° F. | 82,000              | 136,000 | 212   | 41.0          | 31.0        |
|    | B   | do                                                       | 126,000             | 167,000 | 321   | 37.0          | 26.0        |

Y. P. = yield point in pounds per square inch.  
T. S. = tensile strength in pounds per square inch.

B. H. = Brinell hardness number.  
R. A. percent = percent reduction of area.

El. percent = percent elongation in 2 inches.

The improved heat treatment contemplated by the present invention imparts higher mechanical properties to heat treated titanium containing material having compositions within the ranges herein set forth than is obtained by conventional heat treating procedures. Tensile properties are obtained which are higher by about 10,000 to 15,000 pounds per square inch, or even more, than can be obtained by other known methods of heat treatment. The higher tensile properties are obtained without substantial decrease in ductility.

In general, the heat treatment involves a novel aging procedure which comprises a combination of one or more holding periods at predetermined temperature and one or more controlled and critical slow rates of cooling to lower temperatures. The alloys of the present invention need not be and preferably are not quenched prior to aging in order to render them susceptible to age hardening, i. e., the use of a high temperature quench is not necessary. The alloys are usually quenched only when it is desired to have the alloys in the soft condition, i. e., to prevent them from age hardening during cooling following hot working or annealing operations. Alloys of the present invention which are in the "annealed" condition have been quenched or rapidly cooled. The alloys will harden to substantially the same final hardness, regardless of whether they have ever been subjected to any quenching or rapid cooling operation during any stage of processing. As a matter of convenience, in order to render the material soft and easy to straighten, chip and overhaul, as well as to prevent danger of cracking during reheating, rods, billets, and blooms are generally quenched after each hot working operation. The initial temperature of the aging treatment and the amount of time required for the complete treatment is determined by the amount of cold work which the material has received since its last annealing or hot working operation. In practice, the material is preferably held at a temperature of about 1000° F. to about 1225° F. for from about one-half hour to about 16 hours, or more, and subsequently cooled more or less continuously to a temperature of about 900° F. to about 800° F. at a rate not exceeding about 75° F. per hour and

preferably about 50° F. or 25° F. per hour or even less, e. g. 12° F. per hour. While the rate of cooling down to a temperature of about 1100° F. may be more rapid, e. g., 75° F. per hour, the rate of cooling below about 1100° F. should not exceed about 50° F., and should preferably be about 25° F. or less per hour. Theoretically the maximum properties appear to be developed by cooling at not more than about 15° F. per hour down to about 900° F. and at about 4° F. per hour from about 900° F. down to about 800° F. The increase in mechanical properties with decreasing temperature is continuous although at a decreasing rate. Thus, material having the compositions contemplated by the present invention which have been cooled slowly to 900° F. in accordance with the improved heat treatment will have higher properties than would have been developed had the slow cooling been terminated at 1000° F. Below about 800° F. the increase in properties is so slow that for practical reasons the slow cooling is seldom continued below this temperature, and often is discontinued at about 900° F. In commercial applications, the material may be quenched, air cooled or cooled at any convenient rate from the final temperature, e. g., from about 800° F., down to atmospheric temperatures. A quenching operation after the hardening treatment decreases the total time consumed in the heat treatment.

When it was required to increase the physical properties above those obtained by the conventional treatment, it has generally been necessary in the past to "cold tap" the product to meet the required physical properties. This practice resulted in extra cost and also in the splitting of a large percentage of finished products during heat treatment. The improved aging process imparts higher physical properties without having to resort to "cold tapping." The process has been used effectively in aging not only the nickel-copper-aluminum-titanium alloys but has also been used satisfactorily to age harden other nickel products having compositions rendering them age hardenable. Age hardenable nickel products containing aluminum and titanium, or aluminum, or titanium, or aluminum and another age hardening element which have been treated in the improved manner, without being quenched prior to aging, have developed high hardnesses and other high physical properties.

The initial temperature of the improved aging treatment and the amount of time required is considerably affected by the cold worked condition of the material being treated. In general, it is preferred to use lower initial temperatures the greater the amount of cold work. The following examples are illustrative of the preferred procedures which will develop near maximum properties in material with and without various amounts of cold work.

#### EXAMPLE NO. I

Material which is in the soft condition, i. e., hot rolled, annealed, or lightly cold worked, develops near maximum mechanical properties when held for about one-half to about two hours at a temperature within the range of about 1175° F. to about 1225° F., subsequently cooled to about 1100° F. at a rate of between about 25° F. and about 75° F. per hour, preferably about 50° F. per hour, and subsequently cooled at a controlled rate not exceeding 50° F. per hour, preferably about 25° F. or less per hour, to a temperature within the range of about 800° F. to about 900° F.

## EXAMPLE NO. II

Material which has received a moderate amount of cold work, such as half-hard temper strip, cold drawn rod, etc., develops near maximum properties when held within the temperature range of about 1050° F. to about 1100° F. for about 8 to about 16 hours and subsequently cooled at a controlled rate not exceeding 50° F. per hour, preferably about 25° F. or less per hour, to a temperature within the range of about 800° F. to about 900° F., e. g., 800° F. While this procedure is particularly suitable for moderately cold worked material excellent results are also obtained with hot rolled and annealed materials, i. e., materials which have been finished at a sufficiently high temperature during hot rolling or which are in the soft condition such as is obtained by quenching from approximately 1400° F. or higher.

## EXAMPLE NO. III

Material which has received a large amount of cold work, such as spring temper wire and strip, develops near maximum properties when held at a temperature within the range of about 1000° F. to about 1050° F. for from 4 to 8 hours and subsequently cooled at a controlled rate not exceeding 50° F. per hour, preferably 25° F. or less per hour, to a temperature within the range of about 800° F. to about 900° F., e. g., 800° F.

The improved mechanical properties obtained by our method of age hardening are not due to the increased time required for the aging treatment. The following example demonstrates that the higher properties obtained by our improved heat treatment are not the result of longer aging. A one inch diameter hot rolled rod having the composition of the "Alloy F" given in Table XI was treated by our improved method, i. e., aged at about 1080° F. for about 16 hours followed by cooling at about 25° F. per hour to about 800° F. Another rod of identical composition was heat treated in the conventional manner for about 80 hours at about 1080° F. followed by the usual furnace cooling at a rate of about 200° F. per hour. The tensile properties obtained by these two treatments are given in Table X. Prolonged heat treatment in the conventional manner does not produce the higher properties obtained by our improved process.

Table X

| Heat treatment         | P. L. | Y. P. | B. S. | El.  | R. A. |
|------------------------|-------|-------|-------|------|-------|
| Long-time conventional | 64.0  | 94.8  | 153.3 | 25.0 | 47.8  |
| Improved process       | 76.8  | 106.0 | 163.5 | 23.0 | 42.5  |

P. L.=proportional limit in thousand pounds per square inch.

Y. P.=yield point in thousand pounds per square inch.

B. S.=breaking strength in thousand pounds per square inch.

El.=elongation in 2 inches in percent.

R. A.=reduction of area in percent.

For the purpose of giving those skilled in the art a better understanding of the invention, we now give illustrative examples of the compositions, heat treatments, and improved physical properties contemplated by the present invention. Table XI gives the composition of four alloys made in accordance with the principles set forth hereinbefore.

Table XI

| Element  | Alloy C | Alloy D | Alloy E | Alloy F | 5  |
|----------|---------|---------|---------|---------|----|
|          | Percent | Percent | Percent | Percent |    |
| Nickel   | 66.14   | 66.10   | 66.45   | 64.66   |    |
| Copper   | 29.83   | 29.69   | 29.26   | 30.07   |    |
| Aluminum | 2.88    | 2.92    | 2.74    | 2.68    |    |
| Titanium | 0.55    | 0.51    | 0.51    | 0.49    |    |
| Carbon   | 0.14    | 0.18    | 0.13    | 0.14    |    |
| Silicon  | 0.26    | 0.20    | 0.31    | 0.26    |    |
|          |         |         |         |         | 10 |

## EXAMPLE NO. IV

Hot rolled rods, 3/4 inch diameter, having the composition of "Alloy C" were annealed at 1450° F. Some of the rods were then heat treated in the conventional manner for about 16 hours at about 1080° F. and furnace cooled at the usual rate of approximately 200° F. per hour. Another batch of annealed rods was heat treated in the improved manner for about 1 hour at about 1200° F., cooled at a rate of about 50° F. per hour to about 1100° F., and cooled from about 1100° F. to about 800° F. at a rate of about 25° F. per hour. The resulting physical properties are given in Table XII.

25

Table XII

| Heat treat-<br>ment | P. L. | P. S. | Y. P. | B. S. | El.  | R. A. | B. H. N. | 30 |
|---------------------|-------|-------|-------|-------|------|-------|----------|----|
| Annealed            | 16.0  | 23.0  | 37.0  | 94.5  | 43.0 | 65.6  | 156      |    |
| Conventional        | 66.0  | 81.5  | 104.0 | 153.8 | 25.5 | 37.5  | 235      |    |
| Improved            | 82.0  | 98.0  | 117.5 | 163.0 | 21.0 | 32.2  | 302      |    |

P. L.=proportional limit in thousand pounds per square inch.

P. S.=proof stress in thousand pounds per square inch.

Y. P.=yield point in thousand pounds per square inch (0.2 percent off set).

B. S.=breaking strength in thousand pounds per square inch.

El.=elongation in 2 inches in percent.

R. A.=reduction of area in percent.

B. H. N.=Brinell hardness number.

35

## EXAMPLE NO. V

Hot rolled rods, 3/4 inch diameter, having the composition of "Alloy C" were subjected in the as hot rolled and quenched condition to heat treatment in the conventional and improved manner. Conventionally heat treated rods were held for about 16 hours at about 1080° F. and furnace cooled at approximately 200° F. per hour. Rods heat treated in the improved manner were held at about 1080° F. for about 16 hours and then slowly cooled to about 800° F. at a rate of about 25° F. per hour. Some of the resulting physical properties are given in Table XIII.

40

Table XIII

| Heat treat-<br>ment | P. L.* | P. S. | Y. P. | B. S. | El.  | R. A. | B. H. N. | 45 |
|---------------------|--------|-------|-------|-------|------|-------|----------|----|
| As hot rolled       | 30.0   | 36.0  | 45.0  | 96.3  | 43.0 | 68.2  | 159      |    |
| Conventional        | 68.0   | 86.0  | 109.0 | 156.9 | 26.0 | 41.8  | 235      |    |
| Improved            | 85.0   | 99.0  | 119.0 | 166.5 | 24.0 | 37.7  | 311      | 50 |

\*See footnote to Table XII for key.

## EXAMPLE NO. VI

Cold drawn rods, 1.125 inches diameter, having the composition of "Alloy D" were heat treated in the as cold drawn condition in accordance with conventional practice and in accordance with the improved procedure. The conventional process comprised heating to about 1080° F. and holding for about 12 hours, then furnace cooling at a rate of approximately 200° F. per hour. The improved procedure comprised heating to about 1080° F. and holding at that temperature for 70 hours.

65

about 12 hours, and then cooling at a rate of about 25° F. per hour to about 800° F. The physical properties possessed by the rods are given in Table XIV.

5

Table XIV

| Heat treatment   | P. L.* | P. S. | Y. P. | B. S. | EI.  | R. A. | B. H. N. |
|------------------|--------|-------|-------|-------|------|-------|----------|
| 10 As cold drawn | 80.0   | 87.0  | 99.0  | 116.0 | 23.5 | 47.8  | 235      |
| Conventional     | 103.0  | 117.0 | 135.0 | 164.7 | 19.0 | 34.5  | 321      |
| Improved         | 114.0  | 124.0 | 142.0 | 174.0 | 18.0 | 32.8  | 341      |

\*See footnote to Table XII for key.

15

EXAMPLE NO. VII

Strip cold rolled full hard (50%) to 0.250 inch gauge and having the composition of "Alloy E" in Table XI was subjected to the conventional heat treatment while another lot of the same 20 cold rolled strip was heat treated in accordance with the improved heat treatment. The conventionally treated strip was aged at about 1050° F. for about 6 hours and furnace cooled at a rate of about 200° F. per hour. The strip treated in 25 accordance with the improved process was aged for about 6 hours at about 1050° F. and cooled about 25° F. per hour to about 800° F. Table XV gives some of the physical properties of the strip.

30

Table XV

| Heat treatment | P. L.* | P. S. | Y. P. | B. S. | EI.  |
|----------------|--------|-------|-------|-------|------|
| As cold rolled | 68.0   | 81.0  | 128.0 | 139.5 | 10.5 |
| Conventional   | 118.0  | 133.3 | 151.0 | 174.2 | 12.5 |
| Improved       | 130.0  | 143.5 | 164.0 | 183.5 | 12.0 |

\*See footnote to Table XII for key.

The present invention contemplates improved age-hardened articles of manufacture characterized by improved hot ductility during processing and possessing increased strength, hardness, etc., without appreciable decrease in ductility. Typical examples of such articles include rollers and bearing balls, bearings and races therefor, roller 45 chains, non-magnetic drop forgings and tie rods for airplane construction, valve seats and other valve parts, pump rods and the like, pump rod sleeves, pump pistons for high pressures and temperatures, plungers, turbine blades, turbine dia- 50 phragm blading, lock washers, screws and nuts, tools, cutting blades and the like, pins and needles, springs and other resilient elements, airplane instrument parts, nozzles for burners, rods, sheets, strip, wire, bars, rolled shapes, etc.

55 Although the present invention has been described in conjunction with preferred embodiments, it is understood that modifications and variations may be resorted to without departing from the spirit and scope of the invention, as those skilled in the art will readily understand.

We claim:

1. An age hardened wrought article of manufacture made of a nickel-copper alloy comprising 60 25% to 35% copper, 2.3% to 3.4% aluminum, 0.4% to 0.6% titanium, not more than 1% silicon, 0.13% to 0.2% carbon and the balance substantially all nickel, said article having been subjected during processing to mechanical hot working operations and to heat treatment whereby an 65 improved article is produced containing controlled amounts of titanium, aluminum and carbon within the aforesaid ranges while at the same time possessing high mechanical properties, including a hardness of about 300 Brinell, improved 70 resistance to embrittlement when exposed to ele-

vated temperatures for long periods of time and improved freedom from splits and the like compared to an article made of a similar alloy not containing titanium in the aforesaid amounts.

2. An age hardened nickel-copper alloy possessing improved hot malleability comprising 25% to 35% copper, 2.3% to 3.4% aluminum, 0.4% to 0.75% titanium, not more than 1% silicon, 0.13% to 0.2% carbon and the balance substantially all nickel, said alloy containing controlled amounts of titanium, aluminum and carbon within the aforesaid ranges being characterized by improved hot ductility within the hot working range of about 1500° F. to about 2300° F. combined with improved freedom from splits and cracks as compared to a similar alloy not containing titanium in the aforesaid amounts, and said alloy being age hardened to hardnesses in excess of about 265 Brinell hardness number while at the same time possessing improved resistance to embrittlement when exposed to elevated temperatures for long periods of time.

3. An age hardened nickel-copper alloy comprising 10% to 45% copper, 2% to 4% aluminum, at least 0.25% and less than 1% titanium, not more than 1% silicon, 0.05% to 0.3% carbon, and the balance substantially all nickel, said alloy containing controlled amounts of titanium, aluminum and carbon within the aforesaid ranges being characterized by hot ductility within the hot working range of about 1500° F. to about 2300° F. and by improved resistance to embrittlement when exposed to elevated temperatures for long periods of time combined with high hardnesses exceeding about 265 to about 300 Brinell hardness in the aged condition when subjected to an aging process which comprises holding said alloy at temperature within the range of about 1000° F. to about 1225° F. for from about one-half hour to about 16 hours and subsequently cooling substantially continuously to a temperature within the range of about 900° F. to about 800° F. at a controlled rate not exceeding about 75° F. per hour through any temperatures above about 1100° F. and at a controlled rate not exceeding about 50° F. per hour through temperatures below about 1100° F. whereby an improved alloy is obtained possessing improved hot malleability and freedom from splits and cracks while at the same time possessing improved mechanical properties and improved resistance to embrittlement at elevated temperatures.

4. An age hardenable nickel-copper alloy comprising 25% to 35% copper, 2.3% to 3.4% aluminum, 0.25% to 0.75% titanium, not more than 1% silicon, 0.05% to 0.3% carbon, and the balance substantially all nickel, said alloy containing controlled amounts of titanium, aluminum and carbon within the aforesaid ranges being characterized by hot ductility within the hot working range of about 1500° F. to about 2300° F. and improved freedom from splits and cracks after hot working as compared to a similar alloy not containing titanium in the aforesaid amounts while at the same time being age hardenable to hardnesses in excess of about 265 Brinell hardness number and possessing improved resistance to embrittlement in the age hardened condition when exposed to elevated temperatures for long periods of time.

5. In the process of age hardening nickel-copper alloys containing 10% to 45% copper, 2% to 4% aluminum, at least 0.25% and less than 1% titanium, 0.05% to 0.3% carbon, and the balance substantially all nickel, the aging steps

which comprise holding said alloys containing controlled amounts of titanium, aluminum and carbon in the aforesaid ranges at temperature within the range of about 1000° F. to about 1225° F. for from about one-half hour to about 16 hours and subsequently cooling substantially continuously to a temperature within the range of about 900° F. to about 800° F. at a rate not exceeding about 50° F. per hour through any temperatures above about 1100° F. and at a controlled rate not exceeding about 25° F. per hour through temperatures below about 1100° whereby higher hardnesses are imparted to said alloys than by heat treating similar alloys by a process involving furnace cooling said alloys at the conventional slow rate of about 200° F. per hour.

6. In the process of age hardening nickel-copper alloys containing 10% to 45% copper, 2% to 4% aluminum, at least 0.25% and less than 1% titanium, 0.05% to 0.3% carbon, and the balance substantially all nickel, the steps which comprise holding said alloys containing controlled amounts of titanium, aluminum and carbon in the aforesaid ranges at temperature within the range of about 1000° F. to about 1225° F. for from about one-half hour to about 16 hours and subsequently cooling substantially continuously to a temperature within the range of about

900° F. to about 800° F. at a controlled rate not exceeding about 75° F. per hour through any temperatures above about 1100° F. and at a controlled rate not exceeding about 50° F. per hour through temperatures below about 1100° F. whereby higher hardnesses are imparted to said alloys than by heat treating similar alloys by a process involving furnace cooling said alloys at the conventional slow rate of about 200° F. per hour.

7. The process of age hardening nickel alloys containing 10% to 45% copper, 2% to 4% aluminum, at least 0.25% and less than 1% titanium, 0.05% to 0.3% carbon, and the balance substantially all nickel, which comprises heat treating said alloys containing controlled amounts of titanium, aluminum and carbon within the aforesaid ranges in the substantially unquenched condition at predetermined aging temperatures and subsequently cooling substantially continuously at a rate not exceeding 50° F. per hour to minimum effective aging temperatures whereby higher hardnesses are obtained in said alloys than by heat treating similar alloys by a process involving furnace cooling said alloys at the conventional slow rate of about 200° F. per hour.

CLARENCE GEORGE BIEBER.  
MORTIMER PIERCE BUCK.